

3,235,504

## FERRITE MEMORY CORES

Robert S. Weisz, Pacific Palisades, Calif., assignor to Electronic Memories, Incorporated, Los Angeles, Calif., a corporation of California  
No Drawing. Filed Jan. 16, 1963, Ser. No. 251,715  
7 Claims. (Cl. 252—62.5)

This invention relates to ferrite magnetic core material used in the fabrication of magnetic core storage systems, and more particularly to an improved ferrite core material composition.

Attempts to switch presently commercially available ferrite cores at rates such that a full duty cycle occurs within 0.5 microsecond or less, are not quite successful. Cores which are considered "low-zinc" (containing less than 8 percent zinc oxide) in the 30 mil size require in the neighborhood of 500 milliamperes to switch at 0.45 microsecond. Driving these cores at repetition rates on the order of 0.5 megacycle causes the cores to heat up and become unstable, and therefore unfit for use as a storage device. The commercially available cores which are "high-zinc" (containing in excess of 8 percent zinc oxide in the composition), although less prone to overheat due to a lower coercive force, are undesirable for other reasons. These high zinc cores invariably have a rounded hysteresis loop, and associated with this they have a high disturb zero response voltage and a high delta noise.

Because of the foregoing drawbacks of presently available cores, fast switching ferrite memory systems (those having one microsecond or less read/write cycle), are generally built using a "word select" mode of operation instead of a coincident current mode of operation, because in the word select mode of operation there is less disturb current flowing during the operation thereof. However, a "word select" memory is not the most desirable type since in its construction it uses a considerably larger number of semi-conductor devices than are used in a coincident current mode type of memory.

An object of this invention is the provision of a novel formulation for ferrite memory cores which can be operated at full duty cycles at 0.5 microsecond or less without heating up and becoming unstable.

Another object of the present invention is the provision of a new and improved magnetic ferrite core formulation.

Yet another object of this invention is the provision of a unique ferrite memory core formulation which results in a core having a lower noise and lower heating when switched at a higher repetition rate than presently available cores.

The novel features that are considered characteristic of this invention are set forth with particularity in the appended claims. The invention itself, both as to its organization and method of operation, as well as additional objects and advantages thereof, will best be understood from the following description.

It has been found that satisfactory performance at full duty cycles of 0.5 microsecond or less is achieved by using compositions for the ferrite cores which may be expressed as:



where  $x$  varies from .05 to .15 mol. In addition up to .06 or .07 mol of  $\text{ZnFe}_2\text{O}_4$  can replace an additional portion of  $\text{MgFe}_2\text{O}_4$ . Ferrite cores having a formulation falling within the ranges indicated had stability even though switched at repetition rates excess of 0.5 megacycle and also these cores had a much lower undesirable noise characteristic.

In addition to being in the above-compositional range,

a further necessary condition for producing fast switching ferrites in control of the crystal size. The smaller the crystal size the higher the coercive force, but the faster the switching time. Crystal size control may be accomplished by using iron oxide and other constituents of low reactivity or by calcining at a higher temperature than customary and by grinding for a shorter than usual time after calcining. The control of crystal size using these techniques is generally known.

As an illustration of a formulation used for the cores, a typical method for processing the formulation to achieve cores having the desired properties, a formulation consisting of 96 grams of  $\text{MgCO}_3$ , 55.3 grams  $\text{MnCO}_3$ , 112 grams of  $\text{Fe}_2\text{O}_3$  and 22.6 grams of  $\text{SnO}_2$ , was mixed with distilled water and then placed in a ball mill. The mixture was milled for fifteen hours and then removed and the water was dried out. The resulting material was screened through a coarse screen. It was then calcined at a temperature of 1100 degrees C. The calcined material was then ball milled again for five hours. Thereafter a temporary binder, such as polyvinyl alcohol dissolved in water, was added. The mixture was then sieved to retain the material which passed through a 100 mesh per inch screen but not through a 325 mesh per inch screen. The material obtained after the sieving operation was then pressed in a compacting press to a desired shape, such as 50 mils outer diameter, 30 mils inner diameter, and 15 mils thick. The material was then fired. This was done by placing a thin layer of the shaped cores on a platinum sheet. The temperature provided was between 1050 degrees C., and 1350 degrees C. This temperature was maintained for from one-half to five hours, depending upon the coercive force desired. The longer the heating and the higher the temperature the lower the coercive force. Thereafter, the cores were removed and air cooled.

Consider the formulations for 30 mil cores respectively designated as A, B and C, which are shown below:

| 40 | Table I                                                                                                         |  |  |
|----|-----------------------------------------------------------------------------------------------------------------|--|--|
| A. | .70MgFe <sub>2</sub> O <sub>4</sub> · 0.15Mn <sub>3</sub> O <sub>4</sub> · 0.15Mg <sub>2</sub> SnO <sub>4</sub> |  |  |
| B. | .75MgFe <sub>2</sub> O <sub>4</sub> · 0.15Mn <sub>3</sub> O <sub>4</sub> · 0.10ZnFe <sub>2</sub> O <sub>4</sub> |  |  |
| C. | .60MgFe <sub>2</sub> O <sub>4</sub> · 0.15Mn <sub>3</sub> O <sub>4</sub> · 0.25ZnFe <sub>2</sub> O <sub>4</sub> |  |  |

The composition of the 30 mil core identified by A was made in accordance with the teachings of this invention. The composition of the 30 mil cores identified by B and C are compositions for ferrite cores which are commonly used and are commercially purchasable. Table II below shows the electrical and magnetic properties of these cores:

Table II

| 55     | Core | I  | $\mu V_1$ | $dVz$ | $t_p$ | $t_s$ | $\Delta_2$ | $\phi$ |
|--------|------|----|-----------|-------|-------|-------|------------|--------|
| A----- | 450  | 23 | 6         | .22   | .44   | .56   | 5.8        |        |
| B----- | 590  | 35 | 9         | .22   | .46   | .71   | 8.6        |        |
| C----- | 400  | 42 | 12        | .22   | .46   | 1.00  | 10.0       |        |

I=full current drive in milliamperes.

$\mu V_1$ =undisturbed one response voltage in millivolts.

$dVz$ =disturbed zero response voltage in millivolts.

$t_p$ =core peaking time in microseconds.

$t_s$ =core switching time in microseconds.

$\Delta_2$ =stabilized delta noise in millivolts.

$\phi$ =flux in volt-microseconds.

The terminology used as the heading for each column in Table II is intended to be the standard terminology which has been proposed and accepted by the ASTM Committee C-25 for establishing standards for testing and defining terms which apply to the use and testing of non-metallic magnetic cores.

The data found in Table II is given for a temperature of 25 degrees C. at a full driving current as indicated

with rise times at 0.1 microsecond. Partial select current was set at  $0.6 \times$  full drive. Noteworthy for the new material are its low  $dV_z$ ,  $\Delta_2$  (delta noise per pair of cores) and flux (at a nominal drive) which is approximately ten percent greater than the test drive.

Some illustrations of formulations in accordance with this invention, used to make 50 mil cores are shown in the following Table III:

Table III

|                                                                                                                                                     |    |
|-----------------------------------------------------------------------------------------------------------------------------------------------------|----|
| D. .70MgFe <sub>2</sub> O <sub>4</sub> ·.15Mn <sub>3</sub> O <sub>4</sub> ·.05ZnFe <sub>2</sub> O <sub>4</sub> ·.10Mg <sub>2</sub> SnO <sub>4</sub> | 10 |
| E. .715MgFe <sub>2</sub> O <sub>4</sub> ·.15Mn <sub>3</sub> O <sub>4</sub> ·.135MgIn <sub>2</sub> O <sub>4</sub>                                    |    |

Core D as indicated, was driven with a 500 milliampere full drive. A 300 milliampere partial drive was employed. A rise time of 0.15 microsecond was achieved. Core E, the indium core, was driven with the indicated full drive of 450 millamps, and a partial drive of 270 millamps was given. The electrical properties of these two 50 mil core formulations are shown in Table IV.

Table IV

| Core   | I   | $\mu V_1$ | $dV_z$ | $t_p$ | $t_s$ |
|--------|-----|-----------|--------|-------|-------|
| D----- | 500 | 53        | 9      | 0.34  | 0.60  |
| E----- | 450 | 25        | 8      | 0.18  | 0.41  |

The grinding times employed in achieving the formulations indicated above were on the order of those given in the specific illustration. Also, the calcining and firing temperatures were within the ranges given in the specific example, as was the duration of the firing.

There has accordingly been described and shown herein above, a novel, useful and improved composition for magnetic ferrite cores for use in magnetic core memory construction.

I claim:

1. An improved composition for ferrite cores for use in magnetic memory storage devices, said composition consisting of



where  $x$  varies from .05 to .15 mol and where H is a material selected from the group consisting of Mg<sub>2</sub>SnO<sub>4</sub> and MgIn<sub>2</sub>O<sub>4</sub>.

2. An improved composition for a ferrite magnetic memory core which is suitable for use in magnetic memories, said composition consisting of



5 where  $x$  varies from .05 to .15 mol,  $y$  varies from zero up to .07 mol, and H is one of the materials selected from the group consisting of Mg<sub>2</sub>SnO<sub>4</sub> and MgIn<sub>2</sub>O<sub>4</sub>.

3. An improved composition for a ferrite magnetic memory core which is suitable for use in magnetic memories, said composition consisting of



where  $x$  varies from .05 to .15 mol.

4. An improved composition for a ferrite magnetic core which is suitable for use in magnetic memories, said composition consisting of



20 where  $x$  varies from .05 to .15 mol.

5. An improved composition for a ferrite magnetic core which is suitable for use in magnetic core memories, said composition consisting in mols:



25 6. An improved composition for a ferrite magnetic core which is suitable for use in magnetic core memories, said composition consisting in mols:



30 7. An improved composition for a ferrite magnetic core which is suitable for use in magnetic core memories, said composition consisting in mols:



#### References Cited by the Examiner

#### UNITED STATES PATENTS

3,031,406 4/1962 Sacco ----- 252-62.5

#### OTHER REFERENCES

Maxwell et al.: "Magnetic and Crystalline Behavior of Certain Oxide Systems With Spinel and Perovskite Structures," Physical Review, volume 96, No. 6, December 15, 1954, pages 1501-1504.

TOBIAS E. LEVOW, Primary Examiner.

MAURICE A. BRINDISI, Examiner.